

Patented May 29, 1928.

1,671,408

# UNITED STATES PATENT OFFICE.

MICHAEL G. CORSON, OF JACKSON HEIGHTS, NEW YORK, ASSIGNOR TO ELECTRO METALLURGICAL COMPANY, A CORPORATION OF WEST VIRGINIA.

## ALLOY.

No Drawing.

Application filed April 13, 1926. Serial No. 101,811.

The invention is an alloy useful for a variety of purposes and particularly for die-casting.

The properties which are of most importance in metals for die-casting are, ability to give a casting having good mechanical properties, such as strength, hardness and homogeneity; low shrinkage during solidification and cooling; and absence of destructive action on the molds or dies in which the cast is made.

The deterioration which dies for die-casting undergo during use is due to an attack which is in part physical and in part chemical. Both these actions, and particularly the physical one, are reduced in intensity by lowering the temperature at which casting is carried out.

A survey of the field indicates the desirability of copper alloys better adapted for die-casting than those now available. The alloys of copper with aluminum, zinc and tin respectively, have some desirable properties but each is deficient in some important respect. The aluminum bronzes require high casting temperatures and suffer too much shrinkage. The zinc alloys, such as Muntz metal and its known modifications, have desirably low melting points but because of their zinc content they strongly attack all iron alloys suitable for making the molds or dies. The copper-tin alloys, such as admiralty metal, suffer relatively little shrinkage but do not crystallize uniformly during solidification.

The only other binary alloys of copper in which the melting point is progressively lowered with increasing content of the metal alloyed with the copper are the copper-manganese alloys. These alloys exhibit another highly desirable property for the use under discussion, viz, as the manganese content increases and the melting point is depressed, the temperature drop between the beginning and the end of freezing becomes less, until at 34% manganese the melting point is only 875° C. and the molten alloy solidifies at practically constant temperature.

Unfortunately copper-manganese containing about 34% manganese is not sufficiently fluid when molten to produce good castings, especially if the mold is at all intricate, and furthermore the solid metal has poor mechanical properties. By diminishing the manganese content to about 15% to 25%,

the melting point is somewhat raised but the metal is improved in all other respects. An addition of phosphorus or silicon brings about an additional improvement which consists mainly in further increasing the fluidity 60 of the molten alloy. The phosphorus and silicon also have the desirable effect of giving the alloy greater strength when it is heated to temperatures approaching its melting point. A content of about 0.1% to 3% of 65 either element may be used. An alloy containing about 20% of manganese and about 1% of phosphorus or silicon is preferred. Elements other than copper, manganese, phosphorus and silicon may of course be 70 incorporated for special purposes. For example, nickel and tin may thus be added.

The preferred alloy referred to above begins to melt at 890° C. and is completely molten at 905° C. When molten it is sufficiently fluid for the making of intricate castings. It has very little effect on iron molds, chemical action being practically prevented by the film of oxide which forms about the stream of molten alloy as it enters the mold; 80 and both chemical and physical attack are diminished by the relatively low pouring temperature. The preferred alloy has an impact resistance only slightly lower than that of admiralty metal (88% copper, 12% tin, 85 2% zinc) while it registers 136 Brinnell hardness and 22 scleroscope and is therefore considerably harder than either admiralty metal or phosphor-bronze (89.5% copper, 10% tin, 0.5% phosphorus). It also shrinks 90 less than admiralty metal or phosphor-bronze, and these in turn shrink the least of the copper alloys heretofore available. At high temperatures it greatly excels them in strength. It is possible 95 to cast blanks from the phosphorus- or silicon-containing copper-manganese alloys of approximately the size and shape desired in the finished article and then to finish them by light drop-forging, such a 100 procedure being quite impossible with any of the copper-tin bronzes now used for die-casting.

In making the alloys of the invention the phosphorus or silicon is preferably added 105 to the melt before the manganese in order that the metal may be thoroughly deoxidized and oxidation of the manganese prevented.

I claim:

1. A non-ferrous alloy containing about 110

15% to 25% of manganese and 0.1% to 3% of an element having the properties of phosphorus and silicon, with the balance principally copper.

5 2. A non-ferrous alloy containing about 20% manganese and about 1% of an element having the properties of phosphorous and silicon, with the balance principally copper.

10 3. A non-ferrous die-cast article composed of an alloy containing 15% to 25% of man-

ganese and 0.1% to 3% of an element having the properties of phosphorus and silicon, with the balance principally copper.

4. A non-ferrous die-cast article composed of an alloy containing about 20% manganese 15 and about 1% of an element having the properties of phosphorus and silicon, with the balance principally copper.

In testimony whereof, I affix my signature.

MICHAEL G. CORSON.